

Feb. 25, 1947.

B. M. S. KALLING ET AL.

2,416,628

METHOD OF EXTRACTING LEAD FROM LEAD SULPHIDE ORES AND CONCENTRATES

Filed Dec. 4, 1943



Inventors  
BO MICHAEL STURE KALLING,  
SVEN JOHAN WALLDÉN AND  
GUSTAF TANNER

By *Stevens and Davis* Attorneys

## UNITED STATES PATENT OFFICE

2,416,628

METHOD OF EXTRACTING LEAD FROM  
LEAD SULPHIDE ORES AND CONCEN-  
TRATES

Bo Michael Sture Kalling, Djursholm, Sven  
Johan Walldén, Stockholm, and Gustaf Tanner,  
Sundsvall, Sweden, assignors to Bolidens  
Gruvaktiebolag, Stockholm, Sweden, a joint-  
stock company limited of Sweden.

Application December 4, 1943, Serial No. 512,977  
In Sweden March 11, 1941

4 Claims. (Cl. 75—77)

1

Known methods for extracting lead concentrates of high lead content and fine grain can not be employed without some special preparatory treatments which involve certain metallurgical inconveniences as well as considerable cost. A charge for sintering and smelting in a blast furnace should not contain more than 45 to 55 per cent of lead whereas flotation concentrates can be had with a content of more than 80 per cent of lead. If the concentrate has a high content of lead it must be diluted by mixing it with some relatively difficultly fusible material prior to the sintering operation. Melting in a blast furnace also requires such a low content of sulphur in the charge that the sulphur has to be removed in two stages, such as by a double sintering of the whole diluted mixture or of part thereof, or by roasting and sintering the same. The simple open hearth process which can be employed for a coarse material having a high content of lead and a low content of gangue can not be used for flotation concentrates owing to their too low permeability to gases.

It has been proposed to effect smelting of the lead sulphide ore and oxidizing its content of sulphide to metal in a single operation but such proposals have not led to any practical results owing to the reason, among others, that such an operation will result in high losses of lead with the flue gases. This is easily explained from the fact that the vapor pressure of the lead sulphide is 109 millimeters at its melting point, viz. 1114° C., 319 millimeters at 1200° C. and 937 millimeters at 1500° C.

This invention relates to a method for extracting lead from lead sulphide ores or concentrates which consists in smelting the material and oxidizing it under conditions that will cause only such part of the lead sulphide to be oxidized as is required for carrying out the process. The invention is characterized by smelting the material so as to form a solution containing lead sulphide and metallic lead together with sulphides of such impurities as may be formed, and then oxidizing the lead sulphide contained in the solution and forming metallic lead. Metallic lead and lead sulphide are intersoluble at the temperatures in question and the solution possesses a relatively low vapor pressure. Such a solution can be produced and oxidized without the lead sulphide being volatilized to an undesired extent.

The quantity of lead required for producing said solution may either be added to the molten lead sulphide in the form of metal or it may be produced in connection with the smelting of the

2

sulphide. In the latter case the lead may be produced by adding lead oxide, lead sulphate or lead oxide and carbon to the charge according to any of the known reactions as given by the following formulas:



10 It has been found that the smelting and oxidizing operation can be so conducted that the necessary amount of lead oxide and lead sulphate may be obtained by recovering and returning the flue dust formed during the lead extracting operations.

15 The requisite oxidation products may also be added in such a way that part of the lead sulphide is roasted before being added to the smelted lead sulphide. It is to be recommended in this case only to roast the material partially which may be performed at such a low temperature that no sintering will take place, for example in the usual shelved furnace. If lead oxide ore is to be had it may of course be directly smelted together with the sulphide ore.

20 In other words, and with reference to the added lead oxide or lead sulphate referred to in the preceding paragraphs, it will be understood that these compounds may be added as such or in the form of lead dust, in the form of partially roasted lead sulphide ores or in the form of partially roasted concentrates of such ores. Accordingly, these various possibilities are contemplated as coming fully within the scope of the present invention.

25 The volatilization of lead during the smelting operation may be substantially reduced if the smelting of the lead sulphide material is performed in an electric furnace where the quantity of gas which escapes from the mass of material and which carries with it volatilized lead sulphide is relatively small compared to the quantity of gases passing through a furnace heated by combustion gases such as an open hearth furnace.

30 The subsequent oxidizing process may be performed in a converter of a known type where air is blown through the bath containing the mixture of lead and lead sulphide. In employing the usual bessemer process too great losses of lead will be caused by gasification, even at a relatively low content of sulphide. It has also proved difficult to obtain a refractory lining for the furnace which will be resistant to the lead oxide formed during the blowing operation by

the lively motion of the bath. The slag obtained during the smelting operation is relatively poor in lead due to the low solubility of lead sulphide in the slag. During the oxidizing operation the quantity of slag must be kept as low as possible as the lead oxide will very easily form a slag.

Much better results are obtained if the oxidation of the bath is performed in such a way that air is blown along the surface of the bath or obliquely downwards towards its surface. In this way the content of lead sulphide at the surface of the bath will be steadily diminishing so that the volatilization of the sulphide will be less than if the content thereof was distributed evenly throughout the melt, as is often the case when the bessemer process is employed. A thorough mixing in the bath will be obtained in spite of the diminished motion of the bath due to the circumstance that the uppermost layer, being richer in lead, will be heavier than the underlying melted portion and therefore will continually sink downwards and be replaced by a melt richer in sulphur. In this case it will be much easier to make the lining resistant to any attack from such lead oxide as may be formed, because the bath will keep relatively still in the furnace.

As an example of the result which may be obtained by the process according to the present invention, and in order to show how the operation may be performed, the following data are given:

In an electric smelting furnace a bath of slag was heated by passing an electric current through it. During a period of eight hours a charge of the following composition was fed on to the bath:

1020 kilograms of a flotation concentrate comprising 59.5 per cent of Pb, 4.85 per cent of Zn, 3.8 per cent of Fe, 1.09 per cent of Cu and 14.6 per cent of S;  
375 kilograms of a lead slime containing 65 per cent of Pb, about  $\frac{2}{3}$  thereof as sulphate and the rest as oxide;  
9 kilograms of fine coke slack and the required quantity of slag-producing substances.

The charge was fed to the surface of the bath in batches at every 15th second and the previous batch had melted before a new batch was added. The solution of lead in lead sulphide showed the following percentages of ingredients at the middle of the tapping:

| S   | Pb   | Fe  | Zn   | Cu   |
|-----|------|-----|------|------|
| 7.1 | 82.0 | 1.5 | 1.52 | 0.99 |

The metal-containing sulphide melt was poured into a furnace below a covering of molten glass whereupon air was blown against the surface of the bath. The effect was that the glass slag was removed from part of the surface of the bath, bringing the air into direct contact with the melt of lead and lead sulphide. After 45 minutes the slag was drawn off and a new quantity

of glass added. This second batch of slag was removed after still another blowing period of  $1\frac{1}{2}$  hours. After the blowing had been continued for 5 hours in all, there then remained in the furnace a bath of metallic lead covered by a thin layer consisting of a "stone" rich in copper and a slag of glass. 422 kilograms of raw lead could be tapped from the furnace and also 138 kilograms of slag and 242 kilograms of stone and refuse were also obtained. About 40 per cent of the content of lead had been volatilized and thereafter recovered in a gas purifying plant, whereas the remaining lead not accounted for had been retained in the furnace or been removed with the slag from the furnace. Considerably better results may be obtained with still richer lead concentrates.

The accompanying drawing illustrates schematically a flow sheet of the process according to the present invention.

Having thus described our invention, we declare that what we claim is:

1. A method for extracting lead from a material selected from the class consisting of lead sulphide ores and concentrates of such ores, comprising melting said material in admixture with an added substance comprising at least one oxygen-containing compound of lead selected from the class consisting of lead oxide and lead sulphate so as to form a lead sulphide-metallic lead solution having, under the conditions obtaining in the melt, a relatively low vapor pressure as compared to that of lead sulphide alone, and then oxidizing the lead sulphide in the solution thus obtained to form metallic lead.

2. A method as claimed in claim 1, characterized in that said material is melted under conditions such that a minimum of gaseous products is present in the melting zone by melting said material in an electric furnace, thereby reducing the loss of lead by volatilization.

3. A method as claimed in claim 1, characterized in that the oxidation operation is effected by blowing air against the surface of the bath.

4. A method as claimed in claim 1, characterized in that the lead content of the melt is regulated by admixing a carbonaceous reducing material with the charge.

BO MICHAEL STURE KALLING.  
SVEN JOHAN WALLDÉN.  
GUSTAF TANNER.

#### REFERENCES CITED

The following references are of record in the file of this patent:

#### UNITED STATES PATENTS

| Number       | Name     | Date          |
|--------------|----------|---------------|
| 882,193      | Francis  | Mar. 17, 1908 |
| 60 2,043,524 | Williams | June 9, 1936  |
| 723,500      | Thofehrn | Mar. 24, 1903 |

#### OTHER REFERENCES

Hofman, "Metallurgy of Lead," published in 1918, by the McGraw-Hill Book Co. of New York, Pages 72 and 87.